

# UNITED STATES PATENT OFFICE.

FRANKLIN M. REED, OF PITTSBURG, PENNSYLVANIA.

## PAINT.

SPECIFICATION forming part of Letters Patent No. 394,396, dated December 11, 1888.

Application filed March 1, 1888. Serial No. 265,796. (No specimens.)

*To all whom it may concern:*

Be it known that I, FRANKLIN M. REED, of Pittsburg, in the county of Allegheny and State of Pennsylvania, have invented certain new and useful Improvements in Paints; and I do hereby declare the following to be a full, clear, and exact description of the invention, such as will enable others skilled in the art to which it pertains to make and use it.

My invention relates to an improvement in paints; and it consists in a compound composed of stearine, asphaltum, rosin, petroleum, paraffine, rosin-oil, oxide of iron, air-slaked quicklime, and mineral spirits, as will be more fully described hereinafter.

In compounding my paint I take rosin-oil, fifty gallons; asphaltum, seventy-five pounds; stearine, twenty pounds; rosin, ten pounds; paraffine, fifty pounds; air-slaked quicklime, two pounds; oxide of iron, calcined, one hundred and fifty pounds; mineral spirits, twenty gallons. In mixing these ingredients together an iron tank is necessary to contain the mixture when complete and to admit of a sufficient degree of heat. I first put into the tank ten gallons of rosin-oil, seventy-five pounds of asphaltum, twenty-five pounds of stearine, ten pounds of rosin, fifty pounds of paraffine, and two pounds of air-slaked lime. These ingre-

dients are dissolved by the application of heat. 30 When they are thoroughly dissolved and stirred together, forty pounds more of rosin-oil and one hundred and fifty pounds of calcined oxide of iron are added. The compound is then stirred until all of the ingredients are 35 thoroughly mixed, when it is removed from the fire and allowed to cool, when the mineral spirits are added as a drier and the mixture again stirred.

This paint is intended as a water-proof 40 coating, and is especially adapted for covering felt, paper, and canvas roofs. When applied to the hulls of water-crafts, it will not blister or scale, because it is elastic and expands and contracts with the body upon 45 which it is placed.

Having thus described my invention, I claim—

A paint composed of stearine, asphaltum, rosin, paraffine, rosin-oil, oxide of iron, lime, 50 and mineral spirits, in or about in the proportions specified.

In testimony whereof I affix my signature in presence of two witnesses.

FRANKLIN M. REED.

Witnesses:

ALBERT H. SUNSHINE,  
J. S. WEST.

It is hereby certified that in Letters Patent No. 394,396, granted December 11, 1888, upon the application of Franklin M. Reed, of Pittsburg, Pennsylvania, for an improvement in "Paint," errors appear in the printed specification requiring correction as follows: In line 27 the words "twenty-five" should read *twenty*, and in line 32 the word "pounds" should be stricken out and the word *gallons* inserted instead; and that the said Letters Patent should be read with these corrections therein that the same may conform to the record of the case in the Patent Office.

Signed, countersigned, and sealed this 8th day of January, A. D. 1889,

[SEAL.]

D. L. HAWKINS,

*Assistant Secretary of the Interior.*

Countersigned:

BENTON J. HALL,

*Commissioner of Patents.*